

2 Sheets—Sheet 1.

A. HARNICKELL.

Spelter Furnace.

No. 236,221.

Patented Jan. 4, 1881.



Witnesses,

W. A. Bertram

J. L. H. Barclay

Inventor

Albert Harnickell.

by

R. A. Williams.

Attorney.

2 Sheets—Sheet 2.

A. HARNICKELL.  
Spelter Furnace.

No. 236,221.

Patented Jan. 4, 1881.



Witnesses,

W. A. Burham  
Dr. L. W. Bruegg.



Inventor

A. H. Harnickell.  
by  
R. H. Williams.

Attorney.

# UNITED STATES PATENT OFFICE.

ALBERT HARNICKELL, OF BROOKLYN, NEW YORK, ASSIGNOR TO GEORGE A. POPE AND GEORGE B. COLE, OF BALTIMORE, MARYLAND.

## SPELTER-FURNACE.

SPECIFICATION forming part of Letters Patent No. 236,221, dated January 4, 1881.

Application filed March 14, 1879.

*To all whom it may concern:*

Be it known that I, ALBERT HARNICKELL, of the city of Brooklyn, Kings county, State of New York, have invented certain new and useful Improvements in Spelter-Furnaces; and I hereby declare the same to be fully, clearly, and exactly described as follows, reference being had to the accompanying drawings, in which—

10 Figure 1 is a horizontal sectional view of the furnace, and Fig. 2 a vertical sectional view of the same. The left half of Fig. 1 is a section on line 12, the right half on line 34, of Fig. 2, which latter is a section on line 56, Fig. 1. 15 Fig. 3 is a vertical longitudinal sectional view of one of the retort chambers or furnaces; Fig. 4, a similar view, showing the means for heating the retorts simultaneously from without and within. Figs. 5 and 6 are end elevations of the retort-furnaces; Figs. 7, 8, 9, 10, detail views, as hereinafter explained.

My invention has for its object to attain a result on a commercial scale heretofore only reached, and even then but imperfectly, in 25 the laboratory—namely, the production of an article of zinc free from all impurities.

The zinc reduced from zinc-white made from pure ores has heretofore been regarded as the nearest approximation to pure metal; but this 30 source is inadequate to supply the increasing demand for pure zinc to be used in the manufacture of high-grade brass for spinning and cartridge-shells. Besides, the article leaves much to be desired in point of quality, and is 35 very expensive.

My invention consists in certain novel forms of apparatus designed with special reference to the purification of zinc, but also, by reason of certain peculiarities of construction, equally 40 adapted for other purposes, as the metallurgist will readily perceive; and it consists, further, in a novel manipulation of the retorts, designed to render them impervious to and unattacked by the metal or metals, all substantially as hereinafter fully described.

The general arrangement of the apparatus will first be described, each part requiring specific mention being next taken up and fully described in detail, the process or mode of 50 manipulation being finally set forth.

In the accompanying drawings, G is the fire-

box, which is supplied with air from the ash-pit in the usual way, and from which lead the fire-canals J J over bridge-walls H H. The fire passes through combustion-chambers K 55 K, located in the retort-furnaces, from which chambers it passes through openings d d, over the retorts P P, and thence, through similar openings on the opposite side of the retorts, into passages L L, which communicate, by 60 means of smoke-flues M M, with the chimney E.

Q Q are suitable dampers covering the ends of the channels L L.

Each retort-chamber N is divided longitudinally by a hollow pillar-wall, X, upon which 65 rests the retort P, the openings o o o being connected and leading through openings O O into the fire-box above and below the grate, as shown in dotted lines, Fig. 2. The flues o o, from the lateral retort-chambers, meet the vertical flue between the stack E and the grate-chamber, and contiguous to the latter, and from this vertical flue openings O lead, as clearly shown in Fig. 1, opening into the fire-box, one opening being above and the other below the grate. The flues o receive air through 70 openings o' in the outer walls. (See Fig. 3.) By these means a hot blast, as it were, may be supplied to the fire-box, or let into the furnaces through valves k, worked by dampers 75 V, the air being heated in its passage through the channels o o. This hot blast may be used or not, as desired. The valves k cover openings in the masonry partition between the chambers K and the flues o, and are slid back 80 and forth by means of the dampers V, wholly or partly uncovering the openings. The retorts are provided at one end with a charging-lip, A, and at the other with an inclined condensing-pipe, R, which leads to the receivers 85 B, which latter are preferably arranged to be set in the masonry over the smoke-flues M.

Now, as to the construction of the various parts in detail, it may be said the retorts P are made of good fire-clay, and are provided 95 with charging-nozzles A, of any desired shape, at one end, and with condensing-pipes R at the other. These latter are slightly inclined, as shown in Fig. 3, and enter the receivers B. These latter are of suitable external shape 100 and size, and are provided with a partition, S, that is perforated at a point just under the

end of the pipe R. Tap-holes are formed in the receiver near the bottom, and also just above the partition S, for letting out the contents when desired. A water-jacket, a, is applied to the pipe R when it is necessary to lower its temperature.

T is a pipe inserted in the side of the receiver opposite the pipe R, with which it accurately registers, or into which it enters when pushed inward. Its construction is shown in detail in Fig. 7, where f represents a semicircular partition half closing the pipe.

e is a rod carrying a semicircular scraper, f', on its end, adapted to serve, in connection with the partition f, to completely close the pipe T. The end plate of the pipe is provided with a glass or mica window, t, through which the "color" in the retort may be observed. These details of construction are not shown in Fig. 3, a simple discharge-nozzle being shown as inserted in the pipe T.

D, Figs. 8 and 9, is the casting-mold. It is made, by preference, of zinc, and is provided with a cup, I, to receive the metal as it is poured, and a neck, c, leading to the main mold D. On either side of the neck are lugs g, serving as bearings for the skimmer j, Fig. 10. Pins b b on either side of the mold D support it in the water-bath U. The skimmer is provided with lugs j' j', that rest between the lugs g, the part j resting in the neck c, and serving to skim the metal as it flows under it and retain any dross or oxide.

In Fig. 4 is shown the device used for tempering a new retort, pipes C C being made to lead, respectively, into the retort from the fire-flue J, and from it into the smoke-flue M. By these means the retort is heated simultaneously from without and from within, greatly lessening the danger of cracking it.

I proceed to the preparation of the retort for the metallurgical operations as follows: Upon obtaining a bright heat in the retort, I proceed to the manipulation of closing the pores and fire-cracks inside and rendering the retort perfectly metal-proof and capable of holding, in liquid or gaseous state, any or all metals, without leakage or penetration into the substance of the retort. To effect this I make use of the phenomenon occurring in making illuminating-gas when a retort is worked unskillfully or for too long a time—viz., that of "carbonizing." In that process coal-gas is generated, and it is a desideratum to avoid as far as possible its decomposition. I, on the contrary, aim at and obtain a regular and sufficiently thick and smooth deposit of graphitic carbon on the interior of the retort by conducting into it a hydrocarbon gas obtained from coal-tar, tallow, rosin, or other equivalent substance, and maintaining the gas under pressure in the retorts while subjected to a decomposing heat. Small safety-jets l l lead from the retorts, for the escape of the highly hydrogenous products of decomposition of the gas, which are ignited, as shown. In about

forty-eight hours the process is complete. The condenser and receiver are next connected with the retort, and the latter is ready for charging.

In case an alloy or mixture of zinc and iron is to be treated, a thick layer of ordinary carbon is introduced on the bottom of the retort.

In the case of alloys of zinc which fuse with difficulty, such as the zinc-silver scum from Parke's method of extraction, or the bottoms of galvanizers' baths, the same are introduced into the retort by means of a double gate-hopper or similar air-excluding device.

Alloys that are readily fusible are first treated in kettles, the object being a preliminary partial separation of lead, tin, iron, arsenic, &c., by the processes of physicking and liquation. I, however, add any reagents used, such as sulphur, below the surface of the bath, filling them into tubes, which are plunged to the bottom of the kettles, insuring a more perfect distribution of the reagent than is possible by the usual process of stirring, while avoiding certain disadvantages attending the latter method.

The next manipulation takes place in the retort-furnace—viz., that of charging metal. In the matter of composing the charge, in view of traces of impurities left in from the previous operations, the operator avails himself of well-known principles of metallurgy to vary the admixture of fluxes or reagents, according to the nature of the metal under treatment. As the heat in the retort is sufficient to render any alloy of zinc fluid, the operation of charging is repeated at intervals, but not beyond filling the retort half full, nor so quickly as to cool the inside of it seriously. The heat in the chamber is kept at the distilling-point of zinc. In the retort it is, of course, lower during the act of filling in.

Simultaneously with the operation of charging, another manipulation takes place at the rear end of the retort—viz., the long pipe T is pushed through the receiver B into the condensing-pipe R, thus closing the receiver and leaving as the only outlet from the retort the pipe T. This latter may be kept shut by means of a simple outlet-valve, s, or left open to allow of the escape of non-metallic gases, if any are expected to form; but the air must be kept out of it; hence it is better that the valve should close automatically. The result of the operation at this point is the volatilization successively, according to their distilling-points, of all metals in the retort which are volatile below the distilling-point of zinc, such as cadmium, antimony, arsenic, mercury, &c. They condense in the pipe T, which is cool, and are scraped toward its opening by manipulating the scraper f', as explained above. The receiver is thus kept closed until sufficient condensation of zinc in the pipe R gives evidence of the operation with the fugitive metals being completed. Where it is worth while to save any of these metals, as cadmium,

the same is secured separately by keeping the pipe well cleaned of substances condensing previous to its vaporization.

Where poisons, like arsenic, antimony, or mercury, are expected, or their presence in the retort is suspected in any appreciable quantity, all joints must be made absolutely tight, and unless the vapors of such metals are to be condensed, when their proper metallurgy as to condensation comes into play, connection, by a hood or otherwise, must be made between the end of the pipe T and the chimney.

Where an amalgam of zinc and mercury is to be treated, the condenser and receiver must be of wrought-iron and the pipe T end in a vessel of water. The heat is not allowed to reach the full distilling-point of zinc. Zinc, however, will distill over with the mercury in small quantity and lodge in the receiver, in which the heat will be sufficient to continue driving mercury into the cool pipe T. The zinc in the receiver is disposed of for common purposes, and the contents of the retort are tapped for redistillation, or made into paints, since traces of mercury may still remain; the quicksilver will be found pretty pure.

Referring, again, to the regular process at this stage—viz., upon the appearance of solid or liquid zinc in quantity in the extension-pipe T—the next manipulation takes place, viz: the pipe T is drawn out of the condensing-pipe R, so as to leave its small end flush with the inner side of the receiver. Now the zinc in the retort distills over, condensing in the pipe R, which is heated by the great latent heat set free by the zinc in passing from a gaseous to a liquid state, at first sufficiently and afterward more than sufficiently to prevent solidification. The metal runs out of this pipe through the orifice in the false bottom to the warmed bottom of the receiver B, where it accumulates. Irregularities are corrected by the opportunity given by the cool false-bottom part of the receiver and the cooler extension-pipe T being open to the lodgment of zinc dust, oxide, and impurities. When the condensing-pipe R becomes red hot only zinc goes over. At this time the water-jackets *a* are applied around it to reduce its temperature and give it ample capacity to condense all zinc-gas ascending, so that the same shall not be condensed in the receiver or extension-pipe, nor run in a red-hot state into the lower receptacle.

At regular intervals, and before charging again, the manipulation of tapping the receiver takes place. The lower tap-hole is opened and the lower receiver emptied. The resultant zinc is chemically pure. The contents are allowed to cool without chilling them, until the skin, with adhering clay or dirt, can be taken off in one dip.

The next manipulation is that of casting. This is done in the water-mold D, described above, which has previously been polished, and for castings for rolling is set slightly out of its level, so as to yield the usual tapering plate.

The object of the precautions for cooling the zinc taken already in the condenser, the keeping it at moderate heat in the receiver, cooling it before casting, combing it with the automatic comb *j*, and chilling it at the period of its solidification, is not that of rendering each plate or casting suitable for rolling, in respect to which use the chilling would be generally considered fatal with ordinary spelter, but is twofold, tending to one result. The low temperature is to prevent burning of the zinc and its alloying or mixing with any zinc or other metal dust or zinc-white which, through some irregularity, might come in contact with it, thereby preserving chemical purity, the combination of which quality, with calm fusion and solidity of casting, produces for the product of this art the highest known specific gravity of unwrought zinc, equal to that of the common rolled zinc.

The zinc produced and cast in the manner described is eminently adapted for any and all uses, such as for the chemical laboratory, for medicinal uses, for colors, for rolling, drawing and spinning, for galvanic batteries, for coating iron—especially telegraph-wire—for artistic and for large castings, for all alloys with copper—especially for the brass out of which metallic cartridges are stamped; also for fittings to shot and shell and for cast-brass for naval and ordnance purposes.

After tapping, and while the retort is still pretty well filled with metal, it is again charged with about the same quantity of raw material as that of metal tapped from the receiver. The manipulations of the extension-pipe and water-jacket are repeated, the same as when commencing, only now the period of closing the receiver, as dictated by the phenomenon of zinc appearing, is naturally shorter. This process may go on indefinitely in treating material having only traces of other metals besides zinc, as in case with that previously treated in the kettle-furnace. For that containing much iron, copper, tin, or lead not removed before filling into the retort, and for that material which contains precious metals, the process is varied.

When zinc-silver-lead alloy has been charged, when the retort is half full or less, and zinc has ceased to distill over, the condenser is emptied and the heat increased, so as to remove the last traces of zinc. When this is finished the front plate of the retort is tapped and the resulting lead-silver alloy cast into pigs for cupelling, while the zinc, oxide, and dust are removed from the retort and condenser, and accumulated for a final reduction with fine coal in the same retort, the resultant zinc from which operations possibly containing gold and silver, must be used again in the zincing process at the silver-works, while the product of the simple distillation is free of other metals. At the end of an engagement of a retort for precious-metal alloy the retort and receiver are washed out with molten lead, which is also returned to the silver-works. As

compared with the processes of distilling off the zinc from this alloy now practiced, my invention, as bearing thereon, possesses the following advantages, viz: Facility for operating on a large scale in one furnace, with attending economy of plant, of retorts, of fuel, and of labor. The liability of loss from particles of noble metal being buried in the body of the retort is lessened and the durability of the 10 retorts increased.

When copper, lead, tin, &c., are residue in quantity in a retort, they are simply tapped out in front and cast.

When iron alone is expected to be the residue and would form a sow, then, when intending to run the retort empty, the heat is increased to a real white heat; next carbon and fluxes are introduced to melt the iron *in loco*, which done, it is promptly tapped out; but 15 where iron, tin, lead retain zinc in a combination difficult to deal with except by distillation, then upon zinc ceasing to flow the extension-pipe is pushed into the condenser, the water-jacket is put on, and the heat increased 20 to a point which may distill lead, &c. The condensed product, all in the pipe, is not cast, but returned to the kettle-furnace. The residue in the retort is scraped out or dealt with by way of fusion.

I am aware that carbon-lined crucibles are old, and that it is also old to use the carbon from coal-gas retorts in the construction of crucibles. Such I do not claim, nor do I claim 25 the mold hereinbefore described. I have been minute in describing it and its functions in connection with my process and apparatus, because I believe it to be the best form of mold to be used in connection therewith.

What I claim is—

40 1. In combination with the fire-box and stack, the flues J M K L, retort chambers and furnaces N, as set forth.

2. In combination with the common fire-box

G, the retort-furnace wings located at either side of the same and provided with channels 45 J K L and ducts M, leading to the common stack E, the channels L being provided with dampers Q, as set forth.

3. The retort-furnaces N, having openings O O communicating with the fire-box below 50 or above the grate, or both, as described.

4. In combination with the retort P and pipe R, the receiver B, having perforated false bottom S, as set forth.

5. In an apparatus for separating zinc from 55 other metals, the receiver B, having registering condensing-pipes R T, as set forth.

6. In combination with the retort P, the receiver B, having the inclined registering-pipes R T, for the discharge of condensed 60 products and for the inspection of the color in the retort, as described.

7. In combination with the receiver B, the pipe T, having semicircular partition f and scraper f', substantially as described. 65

8. In combination with the retort-furnace N and flues J K L M, the pipes C, connecting the flues M J with the interior of the retorts, as described.

9. The method herein described of rendering metallurgical retorts metal-proof or impervious to the molten metals, consisting in decomposing within the retorts a hydrocarbon gas, whereby the walls of the retorts become coated and impregnated with graphitic carbon, as set forth. 75

10. In an apparatus for the separation of zinc from other metals by distillation, a retort having its interior surface coated with graphitic carbon deposited from a hydrocarbon de- 80 composed within the retort, as set forth.

ALBERT HARNICKELL.

Witnesses:

GEO. A. POPE,  
R. D. WILLIAMS.